

# United States Patent Office

2,705,685

Patented Apr. 5, 1955

1

2,705,685

## PHOTOSENSITIVE PAPER BASE MATERIAL AND METHOD OF MAKING THE SAME

John F. Cipriano, Philadelphia, Pa., assignor to Adelphi Research and Manufacturing Company, Philadelphia, Pa., a firm

No Drawing. Application November 25, 1952,  
Serial No. 322,547

12 Claims. (Cl. 117—34)

The present invention relates to a method of preparing paper prior to the application of photosensitive materials in the manufacture of photosensitive paper, and to the resulting product; and, more particularly, the invention relates to the treatment of paper which is to be coated with photosensitive materials in the manufacture of photoprint paper, such as blueprint paper, brownprint paper, diazo-type print papers, photographic paper, and the like, and to the resulting treated paper.

In the manufacture of photosensitive papers, such as those enumerated above, a sheet of finished paper is coated with a light-sensitive coating. In the manufacture of blueprint paper, for example, the paper is coated with a solution containing an iron salt or salts. In printing with the resulting paper, the paper is exposed to light under an opaque design, then the sheet is washed to remove the portions of the coating which are not affected by the light. The portions which have been affected by the light can be converted to a blue color by the use of a suitable developing solution of, for example, potassium dichromate.

Much work has been done in the past in an attempt to increase the intensity of the dark areas and thus to increase the contrast between dark and light areas in photoprints. A recent advance in this regard is the method described and claimed in U. S. Patent No. Re. 23,510. The process of this patent involves coating a finished sheet of paper with a layer of discrete submicroscopic particles of silica as by applying to the sheet of an aqueous silica sol, that is, a colloidal dispersion of sub-microscopic silica particles in water, followed by drying. While this treatment has the effect of increasing the contrast between the light and dark portions of the photoprint, the method possesses a substantial limitation in that the coating has to be applied to a finished, calendered sheet of paper. The coating cannot be applied to an unfinished sheet of paper before calendering, since calendering destroys the coating. The result of this limitation is that the paper-coaters, that is, those who coat finished paper with photosensitive materials, are forced to apply the silica precoating, whereas it would be much more desirable and economical for many reasons if the paper manufacturers themselves could apply the coating, for example, in the conventional surface sizing tub, before the paper is calendered.

A further limitation possessed by all conventional photosensitive papers, including those treated in accordance with the process of the above-discussed patent, is the tendency for the photosensitive paper to deteriorate upon standing due possibly to the action of the photosensitive chemicals. This seriously reduces storage life in photosensitive papers. Still another limitation of the process of the above-discussed patent is that because a relatively large amount of silica must be applied to the paper in order to achieve the desired results, the tearing and folding properties of the treated paper are deleteriously affected. Furthermore, the silica particles are highly abrasive and this property has been found to exert undue wear on coating and cutting equipment.

It is the principal object of the present invention to provide a method of treating paper of the type which is to be provided with a light-sensitive coating, as the result of which treatment the final photosensitive paper, upon printing and developing, possesses greater intensity of color and/or greater contrast between light and dark areas than conventional photoprints.

Another object of the present invention is to provide a method of treating paper of the type which is to be coated with photosensitive material which treatment may be

2

accomplished as a step in the manufacture of a paper sheet by the paper manufacturers.

Still another object of the present invention is to provide a sheet of paper which, when coated with photosensitive materials, exposed and developed, will provide a print possessing a more intense color and/or a greater contrast between light and dark areas than does conventional photosensitive paper.

A further object of the invention is to provide a pre-treated paper the treated surface of which is capable of adsorbing a greater quantity of photosensitive chemicals than do conventional photosensitive paper bases.

A further object is to provide a treated sheet of paper which, when the photosensitive materials are applied thereto as a coating, is not as readily adversely affected upon storage by the photosensitive chemicals as are conventional photosensitive paper bases, and which, therefore, possesses greater storage life.

A further object is to provide a method of treating paper of the type described wherein no diminution of the tearing and folding properties of the sheet results.

Other objects will become apparent from a consideration of the following specification and claims.

The process of the present invention comprises coating a sheet of paper with a fluid aqueous dispersion of a basic aluminum carbonate gel and drying the resulting coated sheet. (Herein and in the claims the terms "paper sheet" and "sheet of paper" will, unless otherwise qualified, refer to a finished calendered sheet as well as to an unfinished sheet, that is, a sheet of paper which has been subjected to preliminary drying but which has not been subjected to final calendering.) The resulting treated paper thus possesses a coating of dried basic aluminum carbonate gel.

Referring specifically to the coating material employed in accordance with the present invention, it is, as stated, a fluid aqueous dispersion of a basic aluminum carbonate gel. Such a gel is prepared by neutralizing an acid aluminum salt with an alkaline carbonate such as sodium carbonate, sodium bicarbonate, potassium carbonate, and the like. Care is taken during this treatment and in subsequent handling of the gel to avoid the liberation and loss of excessive carbon dioxide from the gel; that is, the basic carbonate first formed is kept cool and wet at all times. The gel, in order to be satisfactory from the standpoint of the present invention, must have a relatively high content of  $\text{CO}_2$ , and generally the gel will contain at least about 0.6 mol of  $\text{CO}_2$  per mol of  $\text{Al}_2\text{O}_3$  and the  $\text{CO}_2$  content may go up to about 1.6 mol per mol of  $\text{Al}_2\text{O}_3$ . Preferably, the gel will contain between about .8 and about 1.2 mol of  $\text{CO}_2$  per mol of  $\text{Al}_2\text{O}_3$ . The gel when made up into an aqueous suspension containing the equivalent of about 4%  $\text{Al}_2\text{O}_3$  will have a pH of 6.0-7.5. At a concentration in water above about 6%  $\text{Al}_2\text{O}_3$ , the gel has the consistency and appearance of cottage cheese and will exhibit thixotropic properties. Such a gel is hydrophilic and disperses readily in water to form a milky suspension.

An example of a gel which is particularly applicable for use in accordance with the present invention are the basic aluminum carbonate gels manufactured by Reheis Company, Inc., and designated P-500, P-1000 and P-2000. Such a gel, which is a colloidal suspension of hydrated particles, is to be contrasted to a sol, such as a silica sol, which is a colloidal suspension of dehydrated particles. The gel is preferably substantially free of other materials which may have an adverse effect in photoprint work. For example, substantial amounts of iron in the coating will be objectionable in making diazotype prints, and chlorides are objectionable in making brownprints. The gels are very reactive. They react with acids more rapidly than usual basic alumina gels and will also neutralize more acid. In this connection, the stated gels manufactured by Reheis Company, Inc. are capable of consuming (as a 4% suspension of  $\text{Al}_2\text{O}_3$ ) 23.5 volumes of 1 N  $\text{HCl}$ .

In applying the gel in accordance with the process of the present invention, the gel will be diluted with water such that the free flowing, fluid suspension is provided. The exact concentration selected will depend upon the properties, including absorption, of the paper and the degree of improvement desired, and the concentration may range from as low as about .1% to as high as about

4% of  $\text{Al}_2\text{O}_3$ . Preferably, the concentration of the gel in the suspension applied to the paper is equivalent to between about 5% and about 2%,  $\text{Al}_2\text{O}_3$ .

The pH of the suspension as applied to the paper is between about 5.5 and about 7. As pointed out above, the pH of the gel will normally be between about 6 and about 7.5 and thus, in certain cases, no adjustment of the pH thereof may be necessary. If adjustment of the pH of the gel is necessary in order to provide the desired pH, conventional acids or acid salts, alkaline materials, as the case may be, may be added to the gel.

In addition, it may be desirable, if the suspension is to stand for any length of time, to incorporate therein a dispersing agent to retard or prevent the settling of the basic aluminum carbonate gel particles. In this connection, a magnesium aluminum silicate sold under the name of "Veegum HV" by the R. T. Vanderbilt Company has been found to be particularly advantageous. Other materials may be included in the suspension for any reason that may be desired. For example, conventional anti-feathering agents, such as resins, gums, and the like, may be incorporated in the suspension.

The suspension may be applied to the paper by any one of a wide variety of means, depending in part upon the particular stage in the manufacture of the paper sheet at which the suspension is to be applied. Where the suspension is to be applied to a finished, calendered sheet, the suspension may be applied by spraying, brushing, by applicator rolls, and the like. Where the suspension is to be applied to the unfinished, uncalendered sheet, in accordance with the preferred embodiment of the present invention, the suspension may be applied by dipping as in the conventional sizing tub or by spraying, brushing, applicator rolls, and the like. In this connection, the suspension may be applied in conjunction with the application of other materials to the paper. For example, a sheet of unfinished paper coming from the first drier section may be first run through a conventional glue sizing tub following which the wet sized sheet may be sprayed with formaldehyde either alone or in conjunction with the suspension of the gel. The suspension may be applied to either the felt or wire side of the sheet, although it is preferred to coat at least the felt side since sensitizing chemicals are normally applied to this side of the sheet. It will be seen from the foregoing, that, depending upon the particular technique employed one or both sides of the sheet may be coated. Following application of the suspension to the paper sheet, the sheet is dried, and, if it has not already been calendered, it may be calendered. The resulting paper may then be sensitized by coating the treated surface of the sheet with sensitizing chemicals in the normal manner.

On the resulting sheet, the basic aluminum carbonate gel coats the fibers thereof. Because of its gel characteristics, the coating possesses a continuous matte structure which fills the voids and coats the fibers of the paper sheet.

The product and method of the present invention possesses many important advantages over prior paper adapted to receive light-sensitive coatings and over the prior method of pretreating such paper referred to above. With respect to the method, one of the primary features thereof is the fact that it may be carried out in the normal equipment conventionally used by paper manufacturers, and thus the process may be carried out by the paper manufacturer as a step incident to the manufacture of the paper sheet. This relieves the manufacturer of photosensitized paper from the burden of precoating the paper, and does not require a separate coating and drying procedure as in the case of silica sol. With respect to the precoated product, it has been found that it results in a higher concentration of photosensitive chemicals being adsorbed on the surface of the paper. This results in a more intense color, particularly in the case of blueprint paper, and also in a greater contrast between light and dark areas in the final developed print. Moreover, it has been found that the coating acts as a buffer which neutralizes acidic photosensitive chemicals which are most often used and which would ordinarily in time cause weakening of the paper. Photosensitive papers made from the treated paper of the present invention, therefore, possess greater shelf-life than do prior photosensitive papers prepared from acidic photosensitive chemicals. This buffering action of the coating also aids in the discharge of unreacted photosensitive chemicals, thus enhancing the contrast between light and dark areas on a finished print.

In addition, the basic aluminum carbonate material possesses unusually high pigmenting values so that the light areas of the treated sheet possess increased brightness. Furthermore, since the suspension applied to the paper is relatively dilute, being preferably on the order of about 1% solids, the folding and tearing properties of the paper need not diminish to any substantial extent as is the case when silica sol, which requires substantially higher concentration, is employed. Finally, the dried coating is much less abrasive than the silica coating so that the undue wear of coating and cutting equipment encountered when silica coating is employed is eliminated.

The present invention will be more readily understood from a consideration of the following specific examples which are given for the purpose of illustration and are not intended to limit the scope of the invention in any way.

#### Example I

To 20 gallons of water are added 20 pounds of basic aluminum carbonate gel (J-500 of Reheis Company, Inc., 10%  $\text{Al}_2\text{O}_3$ ), 6½ ounces of concentrated HCl and 8½ ounces of magnesium aluminum silicate (Veegum HV). This suspension is applied to 2200 yards of paper. The coated paper is then dried. The treated sheet is then coated with a conventional blueprint sensitizing solution and dried in the conventional manner. Blueprints made from the resulting paper are much brighter than the conventional blueprints, the blue being a deeper blue giving greater contrast between the blue portions and the white lines.

#### Example II

To 50 gallons of water are added 40 pounds of basic aluminum carbonate gel (P-500 of Reheis Company, Inc., 10%  $\text{Al}_2\text{O}_3$ ), and 2 pounds of magnesium aluminum silicate (Veegum HV). The pH of the suspension is adjusted to 5.5 with citric acid. 17 pound, 50% rag paper, of the type normally used in making blueprint paper, coming from the first drier section of a paper-making machine is first immersed in the conventional glue sizing tub and the excess sizing is squeezed out by rollers. A formaldehyde solution is then applied to the wire side of the sheet. The above-described suspension, containing also formaldehyde, is run on to the felt side of the paper sheet, and excess suspension is squeezed off by means of squeeze rolls. The sheet is dried and calendered in the regular manner. The treated side of the resulting sheet is then coated in the conventional manner with blueprint sensitizing solution. Blueprints made from the resulting paper give unusually contrasting blue and white portions.

#### Example III

The suspension used in Example II, without formaldehyde, is used in this example. 17 pound, 50% rag paper coming from the first drier section of a paper-making machine is immersed in a tub containing the stated suspension so that the suspension is applied to both sides of the sheet. Excess suspension is squeezed off by means of squeeze rolls, and the sheet is then dried and calendered in the usual manner. The felt side of the treated sheet is then coated in the conventional manner with blueprint sensitizing solution.

In this example, wet strength materials are incorporated in the paper stock before the web is formed, thus eliminating the need for the glue sizing step.

Considerable modification is possible in the selection of additives and in the particular techniques employed in carrying out the present process without departing from the scope of the invention.

#### I claim:

1. The method of treating paper to improve its properties as photosensitive paper base which comprises applying to a sheet of paper a fluid aqueous suspension of a basic aluminum carbonate gel having a pH between about 5.5 and about 7, which basic aluminum carbonate gel has a  $\text{CO}_2$  content of between about .6 mol and about 1.6 mol of  $\text{CO}_2$  per mol of  $\text{Al}_2\text{O}_3$ , and drying the treated sheet.

2. The method of treating paper to improve its properties as photosensitive paper base which comprises applying to a sheet of paper a fluid aqueous suspension of a basic aluminum carbonate gel having a pH between about 5.5 and about 7, which basic aluminum carbonate gel has a  $\text{CO}_2$  content of between about .6 mol and about 1.6 mol of  $\text{CO}_2$  per mol of  $\text{Al}_2\text{O}_3$ , the concentration of

basic aluminum carbonate gel in said suspension being equivalent to between about .1 and about 4%  $\text{Al}_2\text{O}_3$ , and drying the treated sheet.

3. The method of claim 2 wherein the concentration of basic aluminum carbonate gel in said suspension is equivalent to between about .5 and about 2% of  $\text{Al}_2\text{O}_3$ .

4. In the manufacture of paper adapted for use as a base in the preparation of photosensitive paper, the steps of applying to the sheet of paper a fluid aqueous suspension of a basic aluminum carbonate gel having a pH between about 5.5 and about 7, which basic aluminum carbonate gel has a  $\text{CO}_2$  content of between about .6 mol and about 1.6 mol of  $\text{CO}_2$  per mol of  $\text{Al}_2\text{O}_3$ , drying the treated sheet and calendering the sheet.

5. The method of claim 4 wherein the concentration of basic aluminum carbonate gel in said suspension is equivalent to between about .1 and about 4% of  $\text{Al}_2\text{O}_3$ .

6. The method of claim 4 wherein the concentration of basic aluminum carbonate gel in said suspension is equivalent to between about .5 and about 2% of  $\text{Al}_2\text{O}_3$ .

7. The method of making a paper base material adapted for use as a paper base in the manufacture of photosensitive paper which comprises applying to a calendered sheet of paper a fluid aqueous suspension of a basic aluminum carbonate gel having a pH between about 5.5 and about 7, which basic aluminum carbonate gel has a  $\text{CO}_2$  content of between about .6 mol and about 1.6 mol of  $\text{CO}_2$  per mol of  $\text{Al}_2\text{O}_3$ , and drying the treated sheet.

8. The method of claim 7 wherein the concentration of basic aluminum carbonate gel in said suspension is equivalent to between about .1 and about 4% of  $\text{Al}_2\text{O}_3$ .

9. The method of claim 7 wherein the concentration of basic aluminum carbonate gel in said suspension is equivalent to between about .5 and about 2%  $\text{Al}_2\text{O}_3$ .

10. A material suitable as a base sheet in the manu-

facture of photosensitive paper comprising a sheet of paper having a dried coating of basic aluminum carbonate gel thereon, and prepared by applying to said sheet of paper a fluid aqueous suspension of a basic aluminum carbonate gel having a pH between about 5.5 and about 7, and the basic aluminum carbonate gel having a  $\text{CO}_2$  content of between about .6 mol and about 1.6 mol of  $\text{CO}_2$  per mol of  $\text{Al}_2\text{O}_3$ , and drying said sheet.

11. The method of treating paper to provide an improved photosensitive sheet which comprises applying to a sheet of paper a fluid aqueous suspension of basic aluminum carbonate gel having a pH between about 5.5 and about 7, which basic aluminum carbonate gel has a  $\text{CO}_2$  content of between about .6 mol and about 1.6 mol of  $\text{CO}_2$  per mol of  $\text{Al}_2\text{O}_3$ , drying the treated sheet, and applying to the dried treated sheet photosensitive chemicals.

12. In the manufacture of photosensitive paper the step comprising applying photosensitive chemicals to a sheet of paper having a dried coating of basic aluminum carbonate gel thereon and prepared by applying to said sheet of paper a fluid aqueous suspension of a basic aluminum carbonate gel having a pH between about 5.5 and about 7 and a  $\text{CO}_2$  content of between about .6 mol and about 1.6 mol of  $\text{CO}_2$  per mol of  $\text{Al}_2\text{O}_3$  and drying said sheet.

#### References Cited in the file of this patent

#### UNITED STATES PATENTS

|           |                  |               |
|-----------|------------------|---------------|
| 147,833   | Fell -----       | Feb. 24, 1874 |
| 2,085,129 | Stoervener ----- | June 29, 1937 |

#### FOREIGN PATENTS

|        |                     |      |
|--------|---------------------|------|
| 16,358 | Great Britain ----- | 1893 |
|--------|---------------------|------|